

1

3,827,967

**THERMAL CRACKING OF HYDROCARBONS**  
Cornelis Nap, Adriaan van Haarlem, and Emile O. H. M. Ruempol, Amsterdam, Netherlands, assignors to Shell Oil Company, New York, N.Y.  
No Drawing. Filed Aug. 30, 1973, Ser. No. 392,892  
Int. Cl. C07r 3/30; C10g 9/16, 23/00  
U.S. Cl. 208—48 R

4 Claims

## ABSTRACT OF THE DISCLOSURE

In the thermal cracking of hydrocarbons the formation of coke deposits and concomitant carburization of iron containing reaction zone surfaces is retarded by carrying out the thermal cracking operation in a reactor wherein the walls of the reactor in contact with the process flow have been coated with a protective overlayer of a metal selected from the class consisting of aluminum and aluminum alloys melting below 1250° C., said coating preferably having interspersed therein a catalytic anti-coke deposition substance made up of a mixture of iron (III) oxide, chromium (III) oxide and potassium carbonate. The protective overlayer or coating employed in the process of the invention is applied to the walls of the reactor in particulate form in admixture with a soldering flux which liquefies at temperatures below the melting point of the particulate metal and catalyst mixture; the reactor walls are maintained at a temperature at which the soldering flux is liquid for a time sufficient to dissolve a substantial portion of the metal oxide present on the reactor wall surface and the reactor walls are then heated to a temperature sufficient to melt the particulate metal which on cooling and removal of the excess flux forms the protective overlayer of the invention.

## BACKGROUND OF THE INVENTION

### Field of the Invention

This invention relates to an improved process for 40 thermal cracking of hydrocarbons wherein the cycle time between shutdowns due to coke build up in the reaction zone is substantially extended and the detrimental effect of carbon corrosion on reactor lifetimes is substantially reduced. More particularly the invention is directed to a thermal hydrocarbon cracking process wherein coke formation and concomitant carburization of iron containing reaction zone surfaces is retarded by coating the reaction zone surfaces with certain metals and inorganic salts and oxides having protective and/or catalytic activity which form a protective overlayer of superior properties when applied to the reaction zone surface by a stepwise process wherein the reaction zone surface is first subject to the metal oxide dissolving action of a conventional soldering flux prior to laying down of the 55 protective overlayer as a metal melt.

### DESCRIPTION OF THE PRIOR ART

The formation of coke deposits, sometimes called sludge or pitch deposits depending on their specific chemical and physical characteristics, on the reaction zone surfaces of thermal hydrocarbon cracking units has long plagued those engaged in hydrocarbon processing and refining. Due to cost factors and the need for structural strength in the processing equipment, commercial scale thermal cracking units are typically constructed from an iron-containing metal such as stainless steels or other iron-containing alloyed metals. With processing equipment of this metal make up, the problem of coke formation on thermal cracking of hydrocarbon fractions seems to be especially critical since ferrous surfaces have a marked tendency towards coke collection and are susceptible to

2

carburization or carbon corrosion due to diffusion of carbon into the ferrous (typically stainless steel) surface at thermal cracking temperatures. Moreover, since the cracking or reaction zone in most conventional hydrocarbon cracking units comprise a series of tubular reactors or coils operated in parallel, the formation of coke deposits on the reaction zone surface can be quickly lead to inefficient operation and shutdown of the cracking unit due to increasing pressure drop, loss of heat transfer through reactor walls and, ultimately, plug off of the reactor as the coke deposit builds up.

A number of varied means and methods have been suggested to avoid or minimize the problems associated with coke build up in thermal hydrocarbon cracking processes. Most pertinent of these expedients for handling the coking problem are those which are directed to prevention of the initial deposition of the coke deposit. Several methods are described wherein various chemical substances such as benzene sulfonic acid derivatives (U.S. 20 3,105,810), aqueous alkali metal salts (U.S. 2,893,941 and 3,617,478) and even light petroleum distillate in combination with subdivided seed particles of coke itself (U.S. 2,717,865) have been added to the process stream to prevent coke deposition on the reaction zone surfaces. A seemingly larger number of references have been directed to methods or means of treating or coating the reaction zone surfaces or reactor walls to prevent deposition. Thus, U.S. 1,689,363 suggests coating the reactor walls with an iron sulphide layer by treatment with hydrogen sulphide; U.S. 2,263,366 teaches that coke formation is suppressed by coating the reactor walls with zinc oxide using conventional means such as galvanization or spraying with molten metal followed by oxidation of the coating; and U.S. 2,063,596 is directed to coating the reaction apparatus with elemental coatings of iron, chromium, molybdenum and lead by decomposition of a volatile metal compound—e.g., metal carbonyls—on the reaction zone surface. More recently, Belgium Pat. 771-594 has proposed forming a protective film of silicon oxide on the reactor surface by steam treatment of a refractory steel containing less than 1% silicon; Japanese Pat. 47/2,601 has suggested the employment of a gold or gold copper alloy coated reaction zone; and U.S. 45 3,536,776 teaches the employment of a reaction chamber constructed of or lined with a metal-ceramic material containing particles of a catalytically inert, refractory solid material, such as alumina, dispersed in chromium to minimize deposition of carbon on reaction zone surfaces.

Even though the methods described above are numerous and varied, none of the methods seem to meet the tests for a completely satisfactory method. This is because each method seems to suffer from one or more deficiencies in that they either do not inhibit coke formation to a satisfactory degree in practice, or they involve expensive materials of manufacture or materials which must be removed from the process flow or lastly, that they involve difficult and expensive modes of preparation, such as coating with materials melting at very high temperatures, which distract from their viability in commercial practice.

### SUMMARY OF THE INVENTION

65 It has now been found that the formation of carbon deposits and the concomitant carburization of iron-containing reaction zone surfaces in contact with the process flow in a thermal hydrocarbon cracking zone can be substantially retarded by carrying out a vapor phase, thermal cracking of hydrocarbon feedstocks in a reaction zone 70 wherein the iron-containing reaction zone surfaces in contact with the process flow have been coated with an over-

layer of aluminum or aluminum alloy melting below about 1250° C. by a process which comprises:

(1) Coating the iron-containing reaction zone surface with particulate aluminum or aluminum alloy melting below about 1250° C. in intimate admixture with a soldering flux having a melting point below that of the particulate aluminum or aluminum alloy employed;

(2) Maintaining the coated reaction zone surface at a temperature below the melting point of the particulate aluminum or aluminum alloy at which the soldering flux is liquid for a period of time sufficient to allow the soldering flux to thoroughly cover the reaction zone surface and dissolve any metal oxide present thereon;

(3) Heating of the reaction zone surface covered with said liquid flux to a temperature sufficient to substantially melt the particulate aluminum or aluminum alloy;

(4) Cooling of the reaction zone surface to form a solid overlayer of aluminum or aluminum alloy thereon; and

(5) Removing the excess flux from the cooled reaction zone surface.

In a preferred aspect of the process of the invention, which is especially applicable to thermal cracking of hydrocarbon mixtures such as naphtha and gas oil in the presence of steam at temperatures of about 400 to about 1000° C. to yield low molecular weight unsaturated hydrocarbons and gasoline components, a mixture of iron (ferric) (III) oxide, chromium (III) oxide and potassium carbonate is added in particulate form to the admixture of aluminum or aluminum alloy and soldering flux employed in step (1) of the above process. This composite mixture of particulate aluminum or aluminum alloy, ferric (III) oxide, chromium (III) oxide and potassium carbonate in admixture with the soldering flux when subject to the processing steps (1) through (5) described above, will yield an aluminum or aluminum alloy coating having interspersed therein a ferric (III) oxide, chromium (III) oxide and potassium carbonate composite mixture which exhibits both protective properties against carburization of the iron-containing reaction zone surface and superior catalytic activity against coke formation.

#### DESCRIPTION OF THE PREFERRED EMBODIMENTS

The process of the invention in its broad aspects involves an improved process for thermal cracking of hydrocarbons wherein coke deposition or formation on iron-containing reaction zone surfaces and the concomitant carburization of such surfaces in contact with the process flow is substantially retarded. The basic thermal hydrocarbon cracking process contemplated by this invention is the conventional non-catalytic cracking process which is well known to those skilled in the art. Though numerous variations and modifications in terms of equipment design, process flow, and the like are both within the purview of those skilled in the art and within the scope of this invention, the thermal or non-catalytic cracking process of this invention can be described in general terms as the conversion of a hydrocarbon feedstock into hydrocarbons having fewer carbon atoms and/or a greater proportion of unsaturated bonds per molecule than the feedstock composition by passing the hydrocarbon feedstock, which has been optionally preheated, into a reaction zone, optionally in the presence of injected steam, wherein the hydrocarbon feedstock in the vapor state is subject to elevated temperatures and residence times sufficient to crack or thermally convert it into the desired lower molecular weight and/or more unsaturated product.

A broad spectrum of petroleum or other naturally occurring hydrocarbon derived feedstocks may be processed in this basic process, or variations thereof, to yield a variety of hydrocarbon products. Suitable feedstocks include light saturated and unsaturated aliphatic hydrocarbons such as ethane propane butane, butylene pentane, cyclopentane, butadiene and the like; the so called intermediate refinery fractions such as naphthas, kerosenes,

gasolines and gas oils; and the heavier hydrocarbon stocks which can be vaporized in conventional thermal cracking equipment.

While it will be recognized that the temperature and residence time in the thermal cracking reactions zone can vary widely with specific feedstocks composition, desired products and feedstock conversion; best yields are generally obtained through employment of short residence times in combination with high reaction zone temperatures. Typically, reaction zone temperatures ranging from about 400 to about 1500° C. in combination with residence times of from about 5 to less than 0.1 seconds. A preferred aspect of this invention involves thermal cracking of intermediate hydrocarbon fractions such as mixtures of naphtha and gas oil in the presence of steam. In this preferred aspect reaction zone temperatures ranging from about 400 to about 1100° C. are quite suitable with temperatures in the range of about 700 to 900° C. being preferred. The pressures employed in the cracking process may suitably range from a pressure adequate to produce the desired flow through the reaction zone up to slightly elevated pressures of, for example 100 p.s.i. The higher pressures are typically employed in thermal cracking of gas oils or lighter fractions to produce unsaturated products.

The thermal cracking reaction zone typically consists of a series of tubes or coils of diameters ranging between about 5 and 25 cm. which are disposed in a cracking furnace and connected in parallel to the process flow. Due to the severity of the conditions employed in the cracking operation these tubes or coils are typically fabricated out of iron containing alloys such as stainless steel. The substantial benefits derived from this invention are based on employment of a reactor wall made up of an iron-containing metal, accordingly, it is contemplated that the thermal cracking zone, irrespective of its specific configuration will be bounded by reactor walls made up of an iron-containing metal material such as stainless steel.

The substantial benefit of the invention—i.e., substantial retardation of coke formation and concomitant carburization of iron-containing reaction zone surfaces in contact with the process flow—is obtained when the thermal cracking of the hydrocarbon feedstock is carried out in a reaction zone coated on the process side with an overlayer of aluminum or an aluminum alloy melting below about 1250° C., applied via the coating process of the invention. This coating process affords an economical means of applying the protective overlayer which is free of many of the operational difficulties associated with the prior art coatings and coating processes. Moreover, this protective overlayer laid down by this process is sufficiently adherent, tough and uniform that superior protective properties are obtained over extended runtimes in thermal cracking units. Accordingly, this method of coating the iron-containing reaction zone surfaces in contact with the process flow with the protective overlayer described forms an integral aspect of the process of the invention. Briefly stated, the coating process contemplated by this invention is a multistep process which comprises:

(1) Coating the iron-containing reaction zone surface with particulate aluminum or aluminum alloy melting below about 1250° C. in intimate admixture with a soldering flux having a melting point below that of the particulate aluminum or aluminum alloy employed;

(2) Maintaining the coated reaction zone surface at a temperature below the melting point of the particulate aluminum alloy at which the soldering flux is liquid for a period of time sufficient to allow the soldering flux to thoroughly cover the reaction zone surface and dissolve any metal oxide present thereon;

(3) Heating of the reaction zone surface covered with said liquid flux to a temperature sufficient to substantially melt the particulate aluminum or aluminum alloy;

(4) Cooling of the reaction zone surface to form a solid overlaying of aluminum or aluminum alloy thereon; and

(5) Removing the excess flux from the cooled reaction zone surface.

As indicated above, in the first step of the coating process of particulate aluminum or aluminum alloy is employed. The aluminum starting material suitable for use in the invention is a metallic aluminum of reasonably high purity such as that available in commerce from a variety of manufacturers. The aluminum alloys which are useful in the process include all those aluminum alloys which melt below about 1250° C. Examples of such alloyed materials suitably include aluminum alloys of one or more of the following metals: silicon, copper, gold, silver, zinc, tin, lead and iron. Preferably the aluminum component comprises a major portion of the alloyed material with alloys or at least 50% by weight aluminum being preferred and alloys of 70% or more by weight aluminum being most preferred. While the maximum melting temperatures of the alloyed materials should not exceed about 1250° C., the melting point can vary over a wide range below that limit. Typically, alloys containing the preferred proportions of aluminum melt between about 600 and about 1000° C., accordingly melting points in this range are preferred. The particle size of the particulate aluminum or aluminum alloy may also vary within wide limits, with the only real limitation being a practical one as to the maximum particle size which can be uniformly applied as an adherent particulate coating by this method. Typically, the aluminum or aluminum alloy starting materials are applied as powders to the reaction zone surface. Such powders suitably have a mean particle diameter of from 35 to 400 mesh.

The term "soldering flux" comprises the commercially available mixtures which contain a number of chemical compounds which in the liquid state are capable of dissolving metal oxides present as a skin or impurity on the surface of metals. Examples of such chemical compounds include zinc chloride, ammonium chloride, and the so-called brazing fluxes such as alkali metal borates with or without boric acid, alkali metal bifluorides and other halides. Preference is given to the use of a soldering flux which has a melting point in the range of 70° to 100° C. Examples of such preferred fluxes include the organic fluxes such as rosin.

The ratio of the quantity of soldering flux to the quantity of particulate aluminum or aluminum alloy can also be selected over a wide range. Quantities by weight of soldering flux in excess of the quantity of weight of particulate aluminum or aluminum alloy generally show advantages; a weight ratio of soldering flux to metal powder of from 1:1 to 10:1 is very suitable.

In order to achieve good adhesion of the iron-containing reaction zone surface and the admixture described in the first step of the process, it is preferred to activate the reaction zone surface prior to the application of the coating preferably by abrasion and/or pickling. Abrasion may be carried out by sand-blasting or grit-blasting. Once the reaction zone surface has been activated, the admixture of soldering flux and the desired particulate metal composition can be applied to the activated surface by any conventional means such as spraying, painting, shaking and the like.

Second step on the process may take place at any temperature at which the soldering flux flows but at which the metal powder does not melt. If a solid soldering flux is employed it is advisable to select a temperature which is only slightly (about 50° C.) in excess of the flow point of the selected soldering flux in order to avoid excessive oxidation of the carrier metal and the metal powder. If use is made of a liquid soldering flux, this heating may be avoided. The soldering flux is maintained in liquid or fluid state in this step of the process for a time sufficient to dissolve all or substantially all of the metal oxide which is

present on the reaction zone surface. Time periods ranging from less than one minute up to about 30 minutes are generally quite sufficient to accomplish this result.

After the carrier metal coated with the mixture of soldering flux and particulate aluminum or aluminum alloy as described under (1) has been maintained at a temperature at which the soldering flux is liquid but below the melting point of the particulate metal for a short while as described under (2), the reaction zone surface is further heated as specified under (3), preferably to a temperature which is at most 300° C. above the melting point of the particulate metal, this temperature subsequently being maintained for 1-5 minutes. During this treatment the particulate aluminum or aluminum alloy adheres to the reaction zone surface and forms a coating which imparts the desired properties to the iron-containing reaction zone surface.

After heating to melt the metal as specified above, cooling takes place, generally by exposure to the atmosphere. After cooling, excess soldering flux, which is of no further importance in the use of the carrier metal with the applied coating may be wholly or partially removed, if desired, for example by washing off, preferably with warm water.

While the coating process employed in this invention can be utilized to coat the process side of an iron-containing reaction zone surface of any conceivable configuration which might be employed in thermal cracking of hydrocarbons, the process is particularly suitable for coating the internal walls of tubular reactors which are most widely employed in this process. In this preferred aspect, during the application of the coating (steps (1), (2) and (3) of the process described above) the tube is kept rotating around its longitudinal axis. A number of revolutions per minute resulting in a rotational speed of the tube wall of 0.5-5 m./sec. is very suitable. After the admixture of soldering flux and particulate aluminum or aluminum alloy has coated the inside of the tube under the temperature conditions specified under (2), the temperature is raised to the values specified under (3). This need not take place simultaneously over the entire length of the tube, but may very suitably be achieved by moving a heat source (for example a concentric ring burner or an induction heat source) longitudinally along the exterior of the tube. This movement can effectively be carried out at a speed of a few meters per hour (e.g., 1-10 m./hr.). This speed is naturally dependent on such factors as the heat production of the heat source, the desired temperature, the wall thickness and the diameter of the tube. The tube diameter is usually between 5 and 25 cm.

As indicated above, a preferred aspect of this invention involves the substantial retardation of coke formation and concomitant carburization of iron-containing reaction zone surfaces which occurs on thermal cracking of intermediate hydrocarbon fractions such as naphtha and gas oil, or mixtures thereof, in the presence of steam at temperatures of from about 400 to about 1100° C. to yield lower molecular weight unsaturated hydrocarbons such as ethylene and propylene, and gasoline components such as isopentane and 2,3-dimethylbutane. In this application it has been found that an aluminum or aluminum alloy coating applied to the iron-containing reaction zone surfaces in contact with the process flow according to the coating process of the invention gives superior protective results when a composite mixture of ferric (III) oxide, chromium (III) oxide and potassium carbonate is interspersed in the protective coating. These three components ( $Fe_2O_3$ ,  $Cr_2O_3$  and  $K_2CO_3$ ) in combination seem to exhibit superior catalytic anti-coke deposition properties in this thermal cracking process. Accordingly, in this preferred aspect, a mixture of ferric (III) oxide, chromium (III) oxide and potassium carbonate, in particulate form either as individual components or as an intimate admixture, is added to the admixture of soldering flux and aluminum or aluminum alloy employed in

the first step of the coating process of the invention described above. The remaining steps of the coating process (steps (2)–(5) above) are then carried out substantially as described to yield this superior protective coating. The relative proportions of the 3 catalytic anti-coke deposition components based on the sum of the three components may vary widely. Mixtures consisting of 50–70 parts by weight ferric (III) oxide, 25–40 parts by weight potassium carbonate and 1–5 parts by weight chromium (III) oxide are quite suitable with mixtures containing 60–70 parts ferric (III) oxide, 30–35 parts potassium carbonate and 1–3 parts chromium (III) oxide (all by weight) being preferred. This mixture of catalytic anti-coke deposition components is preferably used in a quantity of from 5 to 100% by weight (based on the sum of the weight of the three components) of the total quantity of soldering flux and particulate aluminum or aluminum alloy employed. It is most preferred to employ the 3 catalytic anti-coke deposition components on an approximate equal weight basis with the aluminum or aluminum alloy employed (based on the sum of the weight of three components).

#### ILLUSTRATIVE EMBODIMENT I

A mixture of 0.75 g. aluminum and 3.75 g. soldering flux in powder form was introduced into a test tube of heat-resistant Cr-Ni steel (25% Cr, 20% Ni) having a length of 80 cm. and a diameter of 1 cm. The tube had been given a thorough grit-blasting pretreatment to clean and activate the surface thereof.

The tube was then heated to a temperature of 80–100° C. under rotation with a circumferential velocity between 0.5 and 1 m./sec. Thus an even layer of flux and coating components was formed. Next the aluminum binder material was made to adhere firmly to the wall of the tube by a melting/diffusion process at 850° C. This was effected by moving a heat source from one end of the tube to the other end with a speed of 2–4 m./hr.

The tube subsequently was allowed to cool and excess flux was removed by washing with water.

In order to demonstrate the protecting effect of the coating a mixture of 345 ml./hr. of gas/oil (density 0.82) and 285 ml./hr. of water was fed to the coated tube. The mixture was preheated at 500° C. to achieve complete evaporation, the residence time in the tube was 0.3 sec. based on total mixture in the hot zone, the pressure was 1.7 atm. gauge and the exhaust temperature was 830° C. The product mixture was cooled in conventional equipment. After a run period of 118 hours blockage by deposits was observed in the equipment downstream of the coated tube. The time lapsed before also considerable amounts of carbon were deposited on the internal wall of the tube was 240 hours.

For comparison an uncoated tube was tested under the same conditions. In this case already after 65 hours the operation had to be discontinued because of blockage in the tube.

Another tube was tested after having been aluminum coated in a conventional manner, i.e., by filling the tube with a mixture of blended aluminum powders, and  $Al_2O_3$  followed by heating to a temperature of 800° C.

After only 39 hours the run had to be discontinued due to severe carbon formation.

#### ILLUSTRATIVE EMBODIMENT II

According to the method described in Illustrative Embodiment I a test tube was coated starting from a mixture of soldering flux and an aluminum-silver silicon alloy (15% Ag, 4% Si).

The tube thus coated was tested under the conditions according to the previous Example. It appeared that operation could be continued during 280 hours without clogging problems.

#### ILLUSTRATIVE EMBODIMENT III

Similarly a test was carried out with a tube internally coated as described in Example I, starting from a mixture

of 3.75 g. soldering flux, 1.5 g. aluminum-silver-silicon alloy (16% Ag, 4% Si) and 1.5 g. of a mixture of 64.4 parts by weight of ferric (III) oxide, 2.0 parts by weight of chromium (III) oxide and 33.6 parts by weight of potassium carbonate, the sum being 100 parts by weight.

5 The run time before clogging of the tube occurred was 145 hours.

What is claimed is:

1. An improved process for vapor phase, thermal cracking of hydrocarbon feedstocks wherein the formation of carbon deposits and concomitant carburization of iron-containing reaction zone surfaces in contact with the process flow is substantially retarded by the improvement which comprises carrying out said thermal cracking process in a reaction zone wherein the iron-containing reaction zone surfaces in contact with the process flow have been coated with an overlayer of aluminum or aluminum alloy melting below about 1250° C. by the process of:

20 (1) coating the iron-containing reaction zone surface with particulate aluminum or aluminum alloy melting below about 1250° C. in intimate admixture with a soldering flux having a melting point below that of the particulate aluminum or aluminum alloy employed;

(2) maintaining the coated reaction zone surface at a temperature below the melting point of the particulate aluminum or aluminum alloy at which the soldering flux is liquid for a period of time sufficient to allow the soldering flux to thoroughly cover the reaction zone surface and dissolve any metal oxide present thereon;

(3) heating the reaction zone surface covered with said liquid flux to a temperature sufficient to substantially melt the particulate aluminum or aluminum alloy;

(4) cooling of the reaction zone surface to form a solid overlayer of aluminum or aluminum alloy thereon; and

(5) removing the excess flux from the cooled reaction zone surface.

25 2. The process according to claim 1 wherein the hydrocarbon feedstock is gas, oil or naphtha, or mixtures thereof, and the thermal cracking is carried out at temperatures of about 400 to 1000° C. in the presence of steam.

30 3. The process according to claim 2 wherein a mixture of ferric (III) chloride chromium (III) oxide and potassium carbonate is added in particulate form to the admixture of aluminum or aluminum alloy and soldering flux employed in step (1) of the coating process and the remaining steps of said coating process are carried out to yield an aluminum or aluminum alloy coating having interspersed therein a ferric (III) oxide, chromium (III) oxide and potassium carbonate composite mixture.

35 4. The process of claim 3 wherein the mixture of ferric (III) oxide, chromium (III) oxide and potassium carbonate added to the admixture of aluminum or aluminum alloy and soldering flux in step (1) contains 50–70 parts by weight ferric (III) oxide, 1–5 parts by weight chromium (III) oxide and 25–40 parts by weight potassium carbonate based on the total weight of the 3 component mixture added.

#### References Cited

#### UNITED STATES PATENTS

|           |         |             |           |
|-----------|---------|-------------|-----------|
| 1,689,363 | 10/1928 | Perl        | 208—48 R  |
| 2,063,596 | 12/1936 | Feiler      | 208—48 R  |
| 2,263,366 | 11/1941 | Peck et al. | 208—48 R  |
| 3,536,776 | 10/1970 | Lo          | 260—683 R |

70 DELBERT E. GANTZ, Primary Examiner

G. E. SCHMITRONS, Assistant Examiner

U.S. CL. X.R.

75 23—252 A; 208—106; 260—683 R